

## UNITED STATES PATENT OFFICE.

ALFRED H. THIEME, OF SPRINGFIELD, MASSACHUSETTS.

## PAPER-HANGER'S SIZE.

## SPECIFICATION forming part of Letters Patent No. 737,529, dated August 25, 1903.

Application filed December 27, 1902. Serial No. 136,865. (No specimens.)

*To all whom it may concern:*

Be it known that I, ALFRED H. THIEME, a citizen of the United States of America, and a resident of Springfield, in the county of Hampden and State of Massachusetts, have invented certain new and useful Improvements in Paper-Hangers' Size, of which the following is a full, clear, and exact description.

10 The object of the present improved paper-hangers' size is to produce a new size for the purpose indicated which is comparatively cheap and easily compounded, susceptible of being molded into cakes of suitable size, readily soluble in the ordinary manner for use, and which will not deteriorate in the lapse of any reasonable time.

15 My paper-hangers' size consists in the following ingredients combined in proportions, reckoned in bulk, as follows: ground glue, forty per cent.; sugar, fourteen per cent.; water, forty-one per cent.; isinglass, four and one-fourth per cent.; alum, one-fourth per cent.; salicylic acid, one-fourth per cent.; antisepic material, one-fourth per cent. These ingredients are all dissolved together with water and boiled for about twenty minutes, then allowed to cool and harden, and may then be molded into cakes or cut up into cakes from the mass.

20 In the selection of the ingredients I prefer to use of the isinglass about two and one-eighth per cent. each of red Russian isinglass and white Russian isinglass. For the preservative equal parts, together amounting to one-fourth per cent., of oil of cloves and oil of wintergreen may be used advantageously, but any other equivalent preservative may be employed if preferred.

This paper-hangers' size aside from being 40 one of entire utility and fitness for its purpose is susceptible of more convenient use than paper-hangers' size, which ordinarily is marketed in cans, for the reason that this size, assuming as it does in the manufacture thereof the 45 form of a heavy gelatinous body, permits that the cakes of any size for use in the covering of a given area may be wrapped in paper and distributed among the workmen.

The proportions of the ingredients may be 50 varied somewhat from those given without materially altering the character or efficiency of the size.

Having thus described my improved size, what I claim, and desire to secure by Letters 55 Patent, is—

1. The herein-described size composition containing glue, sugar, water, isinglass, alum, salicylic acid, substantially as described.

2. The herein-described size composition 60 consisting of glue, sugar, water, isinglass, alum, salicylic acid, and an additional preservative material, substantially as described.

3. The herein-described size composition consisting of ingredients in proportions as 65 follows: ground glue forty per cent.; sugar fourteen per cent.; water forty-one per cent.; isinglass four and one-fourth per cent.; alum one-fourth per cent.; salicylic acid one-fourth per cent.; and an essential oil one-fourth per 70 cent., substantially as described.

Signed by me, at Springfield, Massachusetts, in presence of two subscribing witnesses.

ALFRED H. THIEME.

Witnesses:

WM. S. BELLOWES,  
JENNIE V. LEAHY.